

May 26, 1931.

E. GATHMANN

1,806,753

INGOT MOLD

Filed Sept. 15, 1926

*Fig. 1.*



*Fig. 3.*



*Fig. 2.*



*Fig. 4.*



*Fig. 5.*

*Inventor  
Emil Gathmann  
by his Attorneys  
Brodwin & Wright*

## UNITED STATES PATENT OFFICE

EMIL GATHMANN, OF BALTIMORE, MARYLAND

## INGOT MOLD

Application filed September 15, 1926. Serial No. 135,586.

This invention relates to metallic ingot molds of the class having vertical ingot-forming chambers and particularly to molds which are open at top and bottom with walls 5 relatively thick in their lower portion and gradually decreasing in thickness upwards. In pouring or teeming such molds the stream of highly heated molten metal, in the first 10 part of the pouring, strikes the mold chamber walls in the lower portion of the mold chamber with great force and heretofore has often cut into the mold walls and suddenly heated them, thereby setting up strains or 15 stresses which cause cracks or recesses to be formed which often seriously impair the life or efficiency of the mold and make the stripping operation difficult.

The object of my present invention is to prevent the formation of such cracks or recesses and to thus lengthen the life of the mold and to facilitate the stripping operation. Broadly stated, my invention consists in rendering harder and more heat resisting the lower portion of the inner walls of the 25 mold chamber than the mold walls above such lower portion so that said lower walls may receive the impact of the stream of molten metal without being injured while the upper walls retain the desirable characteristics of the cast iron usually employed in 30 making ingot molds.

The accompanying drawings are largely diagrammatic but sufficiently illustrate the best ways now known to me of carrying out 35 my invention.

Figure 1 shows a vertical section of an ingot mold of well known construction with my improvements applied.

Figure 2 is a sectional view of the lower 40 portion of the mold, the section being taken on the line 2-2 of Figure 1.

Figure 3 shows a vertical section of an ingot mold provided with a modified form of my invention.

45 Figure 4 is a sectional view of the lower portion of the mold, the section being taken on the line 4-4 of Figure 3.

Figure 5 is a view similar to Figure 4, the section being taken on the line 5-5 of Figure 3.

The mold shown in Figure 1 has an ingot forming chamber A larger in diameter or cross section in its upper than in its lower portion, the chamber gradually or progressively increasing in width from bottom upwards. The mold is open at top and at bottom and the lower portion of the mold chamber is necked-in by inner mold walls *a* having a concavo-convex contour of the kind shown, described and claimed in my U. S. Patent No. 1,188,751 of June 27, 1916. The bottom opening B of the mold may be closed by a plug C in the usual way or by other suitable means. The walls of the mold are thicker 55 in their lower portion than in their upper part for a purpose now well understood and the mold, for the most part, is made of cast iron of the usual kind. Generally such molds are made of an open grade of Bessemer cast iron containing approximately 60 the following ingredients: silicon 1.25; manganese 0.80; sulphur (under) 0.06; phosphorous (under) 0.20; total carbon 3.75. The contained graphitic carbon usually runs 65 from 3% to 3½%. Cast iron having these 70 characteristics being of a so-called open structure, admirably fulfills an important requirement in ingot molds, viz: it has the capacity of expanding and contracting correspondingly with the variations in temperature 75 incident to the formation of ingots in the mold chamber without fracturing of the mold walls or excessive cracking. But the melting point of such cast iron or mold metal (2,200° F. to 2,300° F.) is relatively low 80 compared with the temperature of steel while being cast, which varies from 2600° F. to 2900° F. and at times is even higher. As a 85 highly heated stream of molten metal enters a mold chamber and strikes against the bottom or lower walls of the chamber, which at first are relatively cool, it often cuts, erodes or even melts the mold walls with which it comes in contact, or so heats said walls as to 90 cause such strains or stresses to be produced as will cause cracks or recesses therein. This has often so changed the contour of the lower portion of the mold chamber as to render 95 the mold inefficient and this has often occurred long before the upper portion of the 100

mold has been seriously impaired. This wearing away of the mold walls is primarily due to cumulative strains produced by continued expansion and contraction of the mold walls caused by temperature changes.

5 If an ingot mold were made entirely of steel, which has a high melting point and hence greater heat resisting qualities than cast iron, the mold walls would be more resistant to the cutting and erosive action of the liquid steel poured into the mold, but steel walls are not suitable for making ingot molds because such steel walls do not so readily expand and contract as do mold walls 10 made of cast iron and therefore they would warp to such an extent as to prevent the removal of the ingot from the mold. Furthermore, the cost of steel molds would be so much greater than cast iron molds that steel 15 could not be used economically. I therefore make the mold principally of cast iron as heretofore and so form or so treat the lower portion of the inner mold walls as to render them harder and more heat resisting than the 20 remaining walls. This may be accomplished 25 in various ways. One way is to form the lower inner mold walls of an alloy of iron with a substance having a high melting point, such as vanadium, molybdenum tungsten, 30 chrome or other such metal. Vanadium for instance, has a melting temperature of approximately 3100° F., which is considerably higher than the temperature of steel when 35 teemed into a mold.

35 It will be understood that the lower portion only of the mold walls should be given the heat resisting qualities above mentioned in order that the upper part of the walls shall have the desirable characteristics of 40 expanding and contracting without cracking, which as before stated, is inherent in gray iron of the kind generally employed in making ingot molds.

Ingot molds of the kind shown are usually 45 cast in sand flasks, bottom end uppermost. In preparing the flask to cast molds of the kind shown in Figures 1 and 2 with my improvements applied, the core of the sand mold is formed in the usual way and a block 50 of high heat resisting material is placed on the core at its upper end so that the molten metal will surround the block when it rises in the flask and will be firmly united therewith when the metal cools and solidifies. The 55 block thus constitutes the upper end of the core during the casting operation. Preferably the block D of high heat resisting material is of the form shown in Figure 1, being tapered as shown and having a serrated upper edge whereby it may be firmly locked to the main mold walls. In the construction 60 shown in Figure 1, the bottom of the mold chamber is formed in the block D and the necked-in portion of the mold chamber is 65 formed in this block. The block may be

formed of an iron alloy of the kind previously described and is, of course, made separately and placed in the sand mold in the manner above explained. The block D in the completed mold is not separable from the mold; 70 it is a permanent part thereof.

The mold shown in Figures 3, 4 and 5 has the lower walls of the cast-iron mold treated to render these walls highly heat resisting. To accomplish this result, the loam or foundry sand composing that portion of the core for forming the lower part of the mold chamber is impregnated and coated with a flour-like metallic dust such as powdered vanadium, molybdenum, chrome and the like made 75 into a paste with molasses and water or other such binder. When the molten metal rises in the sand flask and surrounds the treated core or a part thereof, this treated part of the core adheres to or is absorbed by the 80 cast metal. In this way a lining or a casing of high heat resisting iron or iron alloy is provided in the lower portion of the mold chamber. In Figures 3, 4 and 5 the lining or treated portion of the mold wall is indicated 85 at E. The high heat resisting material should not extend to any considerable extent above the necked-in part of the mold chamber as the desired qualities of ready expansion and contraction of the mold would be impaired 90 if any considerable portion of the walls above the necked-in portion were materially changed. While I have shown in the drawings two practical ways of embodying my invention in ingot molds, it will be understood 95 that the details illustrated and described may be varied without departing from the novel features of my invention.

A cast iron ingot mold made in accordance with my invention has a portion of the matrix side wall of close grained metal comprising double carbides of iron and another metal and where chromium is employed, a portion of the mold wall is impregnated with chromium carbide.

The forming molds in which the ingot molds are cast are of usual construction except as modified in the manner above described. In my U. S. Patent No. 1,719,544 of July 2, 1929, I have claimed the method herein described of forming ingot molds.

I claim as my invention:

1. An ingot mold having a vertical ingot-forming chamber, the inner chamber side walls of which at the lower portion of the mold are formed of an alloyed metal more heat-resisting than the remaining mold walls to the cutting action of liquid steel.

2. A cast iron mold having a vertical ingot-forming chamber the lower inner walls 125 of which are provided with a heat-resisting alloyed portion.

3. As an article of manufacture, a cast iron ingot mold member having a portion of the matrix side wall of close grained metal com- 130

prising double carbides of iron and another metal.

4. An article of manufacture comprising a cast iron ingot mold member having a portion of the wall thereof impregnated with 5 chromium carbide.

5. A cast iron mold having a vertical ingot forming chamber, open at the bottom, in combination with a block of heat resisting material inserted in the lower portion of the 10 mold and which is formed of an alloyed metal more heat resisting than the remaining mold walls to the cutting action of liquid steel.

In testimony whereof, I have hereunto subscribed my name.

15 EMIL GATHMANN.

20

25

30

35

40

45

50

55

60